

[54] **SPECTRALLY SENSITIZED SILVER HALIDE PHOTOGRAPHIC EMULSION**

[75] Inventors: **Keisuke Shiba; Haruo Takei; Akira Sato**, all of Kanagawa, Japan

[73] Assignee: **Fuji Photo Film Co., Ltd.**, Minami Ashigara-shi, Kanagawa, Japan

[22] Filed: **Sept. 28, 1971**

[21] Appl. No.: **184,604**

[30] **Foreign Application Priority Data**

Sept. 28, 1970 Japan..... 45/84532

[52] U.S. Cl..... **96/126, 96/137, 96/140**

[51] Int. Cl..... **G03c 1/14, G03c 1/22**

[58] **Field of Search**..... 96/124, 140, 126

[56] **References Cited**

UNITED STATES PATENTS

2,430,558 11/1947 Carroll et al..... 96/124

**FOREIGN PATENTS OR APPLICATIONS**

1,019,418 11/1957 Germany ..... 96/140

*Primary Examiner*—Norman G. Torchin

*Assistant Examiner*—M. F. Kelley

*Attorney*—Sughrue, Rothwell, Mion, Zinn and Macpeak

[57]

**ABSTRACT**

Silver halide emulsions containing a supersensitizing combination of at least one sensitizing carbocyanine dye and at least one merocyanine dye containing a tetrazole nucleus giving a high white light sensitivity or red sensitivity.

**17 Claims, 6 Drawing Figures**

**FIG. 1****FIG. 2****FIG. 3****FIG. 4****FIG. 5****FIG. 6**

## SPECTRALLY SENSITIZED SILVER HALIDE PHOTOGRAPHIC EMULSION

### BACKGROUND OF THE INVENTION

#### 1. Field of the Invention

This invention relates to a spectrally sensitized silver halide photographic emulsion and more particularly to a silver halide photographic emulsion prepared by the combined use of at least more than two kinds of sensitizing dyes to obtain a high white light sensitivity or red sensitivity.

The photographic sensitive materials are required to have high sensitivity at the specific wavelengths different from each other according to the purpose for use.

#### 2. Description of the Prior Art

It has been well known in the art that for making such photographic sensitive materials certain kinds of sensitizing dyes are added to a silver halide photographic emulsion to raise the sensitivity in the region of wavelengths longer than the region of wavelengths of sensitivity intrinsic to said silver halide; that is, the art of spectral sensitization. Usually more than two kinds of sensitizing dyes are used together, generally, for photographic sensitive materials having panchromatically sensitized spectral sensitivity in order to obtain a desired spectral sensitivity distribution.

Many of the sensitizing dyes, however, bring about the lowering of the sensitivity of the emulsion in the intrinsic sensitivity region thereof, i.e., desensitization, while they bring about spectral sensitization. Therefore, it is quite advantageous to use at least two kinds of sensitizing dyes, which are in a supersensitizing relation to each other and do not accompany desensitizing action.

### SUMMARY OF THE INVENTION

The object of this invention is to lower the desensitizing action and to raise both the sensitivity intrinsic to silver halide and the panchromatically sensitized spectral sensitivity by using at least two kinds of sensitizing dyes.

The second object of this invention is to improve the image quality of the spectrally sensitized photographic sensitive material. Generally, the sensitizing dyes affect the development of the photographic emulsion and, in many cases, lower the quality of the photographic image. Especially, cationic dyes affect the infectious development, which is employed for photographic plate making, and deteriorate the dot quality obtained. Therefore, it is also the object of this invention to obtain high panchromatic sensitivity by supersensitization using a restricted cyanine dye and another merocyanine dye, which have little effect on infectious development, and to obtain good dot quality, which is difficult to obtain by supersensitization using more than two kinds of cyanine dyes together.

Merocyanine dyes are generally adsorbed flat on silver halide to prohibit the formation of the J aggregate of the carbocyanine dye and, as a result thereof, lower the red sensitivity extremely. One of the characteristics of this invention is the discovery of a method for strengthening the formation of the J aggregate of the restricted carbocyanine by strictly selecting the chemical structure of the merocyanine dye.

Other objects and advantages will become apparent from the following discussion.

The object of this invention is accomplished by the combined use of at least one sensitizing carbocyanine dye having two heterocyclic nuclei selected from the group consisting of a benzothiazole nucleus, a benzolelenazole nucleus, a  $\beta$ -naphthoselenazole nucleus, and a  $\beta$ -naphthothiazole nucleus, the meso-position of said dye being substituted with a methyl or ethyl group and, preferably, at least one of the N-substituents of said heterocyclic nuclei being a sulfo alkyl group or a carboxy alkyl group. More specifically, we are speaking of sensitizing dyes of the following general formula (I), and at least one merocyanine dye, wherein a tetrazole derivative nucleus and a merocyanine nucleus are connected through a dimethine chain, more specifically, sensitizing dyes of the following general formula (II):



wherein  $R_1$  and  $R_2$  each represents a lower alkyl group, such as methyl, ethyl, propyl, gamma-sulfopropyl, gamma-sulfobutyl, delta-sulfobutyl, beta-hydroxyethyl, beta-carboxyethyl, allyl group, etc.;  $A$  represents a lower alkyl group, preferably a methyl or an ethyl group;  $Z_1$  and  $Z_2$  each represents the non-metallic atoms necessary to complete a benzothiazole, benzolelenazole, beta-naphthoselenazole, or beta-naphthothiazole nucleus, which may be substituted with a halogen atom, such as chlorine, bromine, etc., a lower alkyl group, such as methyl, ethyl, etc., an alkoxy group, such as methoxy, ethoxy, etc., an alkoxy carbonyl group, such as methoxycarbonyl, ethoxycarbonyl, etc., an aryl group, such as phenyl, toluyl, etc.;  $X_1$  represents an anion, such as chloride, bromide, iodide, methylsulfate, p-toluenesulfonate, etc.;  $m$  is 0 or 1, and  $m = 0$  if an intermolecular salt is formed with  $R_1$  or  $R_2$ ;



wherein  $R_3$  and  $R_4$  each represents a lower alkyl group, such as methyl, ethyl, n-propyl, gamma-sulfopropyl, gamma-sulfobutyl, delta-sulfobutyl, beta-hydroxyethyl, delta-carboxybutyl, allyl, etc.;  $B$  represents a lower alkyl group, such as methyl, ethyl, etc., or an aryl group, such as phenyl, toluyl, etc.;  $Z_3$  represents  $=N-R_5$ , oxygen or a sulfur atom; and  $R_5$  being a lower alkyl group, such as an ethyl and beta-hydroxyethyl. In the above, the alkyl moiety of the lower alkyl group has preferably up to five carbon atoms. The "merocyanine nucleus" is defined as a heterocyclic nucleus containing a



group (refer to C. E. Mees, "The Theory of the Photographic Process," Revised Edition, pages 415 to 420).

## DETAILED DESCRIPTION OF THE INVENTION

The cyanine dyes of this invention having the general formula (I) have their maximum sensitization part between 595 and 690 nm, and many of them have high red sensitivity. Some of the sensitizing dyes having the general formula (II) have their maximum sensitization part between 460 and 560 nm, and others do not exhibit remarkable spectral sensitization action, even when used together with a silver iodide emulsion.

The red sensitivity arising from the sensitizing dye of the general formula (I) is further raised, the white light sensitivity is remarkably raised and the silver halide photographic emulsion, which almost does not cause intrinsic desensitization, can be obtained by the combined use of at least one of the sensitizing dyes of the general formula (I) and at least one of the sensitizing dyes of the general formula (II), which have the said characteristics. Above all, the combination of meso-methyl-carbocyanine, being one of the sensitizing dyes represented by the general formula (I), and the sensitizing dye of the general formula (II) wherein  $Z_3$  is sulfur, remarkably raises the white light sensitivity and red sensitivity, and brings about remarkable maximum sensitization around 630 nm. This shows that the dye having the general formula (II) remarkably strengthens the J-band of the J-band type dye of the carbocyanine sensitizing dyes represented by the general formula (I). This is one of the unique characteristics of this invention. The combination of the dye represented by the general formula (I) (e.g., meso-ethyl-thiacarbocyanine) and the sensitizing dye represented by the general formula (II) wherein  $Z_3$  is an oxygen atom rather sensitizes while strengthening the J-band of the J-band type dye without changing the spectral sensitivity distribution thereof. This is effective for the red sensitization for the red-sensitive layer of color photography. The tendency of the J-band strengthening, of the supersensitizing action and of the effect of prohibiting the desensitization is not injured by using orthochromatic sensitizing dyes, such as 2,2-cyanine, pseudocyanine, and the like.

The sensitizing dyes of the general formula (I) do not deteriorate the dot quality obtained by the infectious development employed for the sensitive material for print plate making in proportion to the fact that they strongly and spectrally supersensitize to the relatively long wavelength of 690 nm. The application of the known supersensitizing art using cyanine dyes together in order to raise the spectral sensitivity badly deteriorates the dot quality. For example, the application of the supersensitizing art described in the specification of U.S. Pats. Nos. 2,533,426, 2,688,545, and 2,751,298, the specification of German Pat. No. 1,547,641, the specification of German Patent Prepublication No. 1,813,001, Japanese Patent Publication No. 16169/68 and No. 4132/68 are disadvantageous because of the reason described above.

The merocyanine dye represented by the general formula rather strengthens the infectious development, and is useful to obtain good dot quality. Accordingly, the supersensitizing art of this invention is useful especially for the panchromatic sensitization of the sensitive material for printing plates which are to be subjected to the treatment of infectious development.

The effects brought about by the groups  $R_3$ ,  $B$  and  $R_4$ , the region of which is concretely mentioned before, are

not so important. Especially when  $R_4$  represents a substituted alkyl group, there will not be such a difference in the effect whether or not an acid group of sulfo or carboxy group is introduced.

Examples of the sensitizing dyes used in this invention are illustrated as follows, but the sensitizing dyes used in this invention are not restricted to these examples only. Sensitizing Carbocyanine Dyes:





**Sensitizing Merocyanine Dyes:**



30 Those skilled in the art can readily synthesize the sensitizing carbocyanine dyes to be used in this invention according to the description in the specification of U.S. Pat. Nos. 2,238,231, 2,503,776 and 3,177,210, German Pat. Nos. 929,080 and 1,072,765, etc., and the sensitizing merocyanine dyes according to the description in the specification of German Pat. No. 1,019,418.

35 The spectral sensitization method of this invention is useful for the spectral sensitization of the gelatinosilver-halide photographic emulsion. It is also useful for the emulsion containing a hydrophilic polymer, other than gelatin, such as agar collodion, water-soluble cellulose derivatives, polyvinyl alcohol, polyvinylpyrrolidone copolymer and other synthesized hydrophilic resin, natural hydrophilic polymer, gelatin derivatives, and the like.

40 The photographic emulsion to be used in this invention is suitably a mixed silver halide comprising at least two of silver chloride, silver bromide and silver iodide. To produce the spectrally sensitized photographic emulsion in this invention, the sensitizing dye according to this invention is introduced into a photographic emulsion according to a conventional method. Usually, dyes are dissolved in a solvent, such as methanol, ethanol, water, cellosolve, water-soluble ketones, etc., and added to an emulsion. Alternatively, dyes may also be dissolved in an oil, slightly soluble in water, then added to water or a hydrophilic colloid to disperse the same.

45 The mol ratio of the sensitizing carbocyanine to the sensitizing merocyanine to be contained in the emulsion can vary widely from 9:1 to 1:9 depending upon the effects desired. The amount of each of the dyes is preferably in the range of from  $1 \times 10^{-6}$  to  $1 \times 10^{-3}$  mol per mol of silver according to the character of the emulsion employed.

50 The photographic emulsion of this invention can be subjected to further hypersensitization and other supersensitization in the known manner. In the production, conventional additives, such as chemical sensitizers,

stabilizers, antibronzing agents, hardeners, surface active agents, antifoggants, plasticizers, development accelerators, color couplers, fluorescent brightening agents, may be contained in the photographic emulsion of this invention in a conventional manner.

The photographic emulsion of this invention may be coated in a common manner on a suitable support, such as a glass plate, film of a cellulose derivative, film of a synthetic resin, Baryta paper, resin-coated paper, etc.

A better understanding of the present invention will be attained from the following examples, which are merely intended to be illustrative and not limitative thereof.

Examples

A silver halide photographic emulsion was prepared by adding separately the dye of this invention illustrated before and to be used in this invention independently to a silver bromoiodide emulsion (AgI:AgBr = 7 mols:93 mols). On the other hand, a silver halide photographic emulsion containing both the carbocyanine dye and the merocyanine dye was prepared.

Each of these emulsions was coated on a triacetylcel-

lulose film base and dried, then exposed to white light using 64 Lux daylight (corresponding to 5,400° K) and at the same time exposed through a red filter (made by Fuji Photo Film Co., Ltd.) which transmits light of

wavelengths longer than 580 nm, or a blue filter which transmits light of wavelengths lying between 400 and 490 nm and has its maximum percent transmission at 450 nm, and developed at 20° C for 8 minutes. The developer used has the composition given in Table 1.

10

TABLE 1  
The Composition of the Developer

|    |                  |       |
|----|------------------|-------|
| 15 | Metol            | 2 g   |
|    | Sodium sulfite   | 100 g |
|    | Hydroquinone     | 5 g   |
|    | Borax            | 2 g   |
|    | Water to make up | 1 l.  |

20 In the following Table 2, the resulting white light sensitivity and red sensitivity obtained by the independent addition of the sensitizing dyes illustrated before and/or the combined addition thereof and the intrinsic sensitivity relative to that of the starting emulsion are given.

25

30

35

40

45

50

55

60

65

Table 2

| Exper-<br>imen-<br>tal<br>No. | Ex-<br>am-<br>ple<br>No. | Sensitizing dye-<br>Amount of dye<br>added<br>( $10^{-5}$ mol/kg of<br>emulsion) | Emul-<br>sion | Maximum<br>sensi-<br>tiza-<br>tion<br>(nm) | Rel-<br>ative<br>white<br>light<br>sensi-<br>tivity | Rel-<br>ative<br>red<br>sensi-<br>tivity | In-<br>tri-<br>n-<br>sic<br>sensi-<br>tivity | Spec-<br>tro-<br>gram |
|-------------------------------|--------------------------|----------------------------------------------------------------------------------|---------------|--------------------------------------------|-----------------------------------------------------|------------------------------------------|----------------------------------------------|-----------------------|
| 1                             | 1                        | A (2)                                                                            | AgBr<br>/I    | 600                                        | 90                                                  | 35                                       | 94                                           |                       |
|                               |                          | A (4)                                                                            |               | " 630                                      | 100                                                 | 90                                       | 90                                           | Fig.1                 |
|                               |                          | A (8)                                                                            |               | " 632                                      | 130                                                 | 120                                      | 80                                           | Curve 5               |
|                               |                          | 1 (2)                                                                            |               | " 540                                      | 82                                                  | 0                                        | 100                                          |                       |
|                               |                          | 1 (4)                                                                            |               | " 540                                      | 88                                                  | 0                                        | 116                                          | Curve 1               |
|                               |                          | 1 (8)                                                                            |               | " 540                                      | 102                                                 | 0                                        | 120                                          |                       |
|                               | 1                        | A (4) 1 (4)                                                                      |               | " 632                                      | 140                                                 | 120                                      | 120                                          |                       |
| 2                             | 2                        | A (8) 1 (4)                                                                      |               | " 632                                      | 170                                                 | 146                                      | 120                                          | Curve 6               |
|                               |                          | 11 (4)                                                                           |               |                                            |                                                     |                                          |                                              |                       |
| 3                             | 3                        | A (4) 1 (4)                                                                      | "             | 630                                        | 164                                                 | 120                                      | 116                                          |                       |
|                               |                          | 12 (4)                                                                           |               |                                            |                                                     |                                          |                                              |                       |
| 4                             | 4                        | 9 (2)                                                                            | "             | 542                                        | 80                                                  | 0                                        | 94                                           |                       |
|                               |                          | 9 (4)                                                                            |               | 542                                        | 84                                                  | 0                                        | 100                                          |                       |
|                               |                          | 9 (8)                                                                            |               | 542                                        | 86                                                  | 0                                        | 100                                          |                       |
| 5                             | 4                        | A (4) 9 (4)                                                                      | "             | 632                                        | 120                                                 | 100                                      | 100                                          |                       |
|                               |                          | A (8) 9 (4)                                                                      |               | 632                                        | 150                                                 | 120                                      | 100                                          |                       |
|                               |                          | 7 (2)                                                                            |               | 540                                        | 90                                                  | 0                                        | 110                                          |                       |
|                               | 5                        | 7 (4)                                                                            | "             | 540                                        | 96                                                  | 0                                        | 116                                          |                       |
|                               |                          | 7 (8)                                                                            |               | 540                                        | 100                                                 | 0                                        | 116                                          |                       |
| 6                             | 5                        | A (4) 7 (4)                                                                      | "             | 610/630                                    | 120                                                 | 100                                      | 105                                          |                       |
|                               |                          | A (4) 7 (8)                                                                      |               | 610                                        | 150                                                 | 100                                      | 116                                          |                       |
|                               |                          | 8 (2)                                                                            |               | 530                                        | 74                                                  | 0                                        | 90                                           |                       |
|                               | 6                        | 8 (4)                                                                            | "             | 530                                        | 76                                                  | 0                                        | 88                                           |                       |
|                               |                          | 8 (8)                                                                            |               | 530                                        | 76                                                  | 0                                        | 88                                           |                       |
|                               |                          | L (2)                                                                            |               | 600                                        | 70                                                  | 25                                       | 94                                           |                       |
|                               |                          | L (4)                                                                            |               | 630                                        | 90                                                  | 60                                       | 88                                           |                       |
|                               |                          | L (8)                                                                            |               | 630                                        | 110                                                 | 90                                       | 80                                           |                       |
|                               | 6                        | L (4) 8 (4)                                                                      | "             | 628                                        | 100                                                 | 68                                       | 88                                           |                       |
|                               |                          | L (8) 8 (4)                                                                      |               | 628                                        | 125                                                 | 100                                      | 80                                           |                       |

Table II—Continued

| Experimen- | Ex- | Sensitizing dye- | Emul-         | Maximum     | Rela- | Rela- | In-    | Spec-             |
|------------|-----|------------------|---------------|-------------|-------|-------|--------|-------------------|
| tal        | am- | Amount of dye    | sion          | sensi-      | tive  | tive  | tri-   | tro-              |
| No.        | ple | added            |               | ti-         | white | red   | sensi- | gram              |
| 7          | B   | B (2)            | AgBr<br>" / I | 655         | 95    | 75    | 85     | Fig.6<br>Curve 15 |
|            |     | B (4)            |               | 660         | 110   | 135   | 88     |                   |
|            |     | B (8)            |               | 665         | 130   | 170   | 78     |                   |
|            |     | 6 (2)            |               | 535         | 80    | 0     | 110    |                   |
|            |     | 6 (4)            |               | 535         | 100   | 0     | 110    |                   |
|            |     | 6 (8)            |               | 545         | 107   | 0     | 96     |                   |
|            | 7   | B (4)            | 6 (4)         | 660         | 135   | 175   | 88     | Curve 16          |
|            |     | B (8)            |               | 665         | 160   | 210   | 80     |                   |
| 8          | J   | J (2)            | "             | 600         | 85    | 30    | 100    | Fig.4<br>Curve 10 |
|            |     | J (4)            |               | 630         | 100   | 88    | 100    |                   |
|            |     | J (8)            |               | 630         | 128   | 105   | 98     |                   |
|            | 8   | J (4)            | 6 (4)         | 630         | 135   | 108   | 110    | Curve 11          |
|            |     | J (4)            |               | 632         | 140   | 100   | 110    |                   |
| 9          | C   | C (4)            | "             | 654         | 100   | 100   | 95     | Fig.2<br>Curve 3  |
|            |     | C (6)            |               | 658         | 108   | 120   | 92     |                   |
|            |     | C (8)            |               | 660         | 110   | 130   | 90     |                   |
|            |     | 2 (2)            |               | "           | 70    | 0     | 100    |                   |
|            |     | 2 (4)            |               | "           | 76    | 0     | 105    |                   |
|            |     | 2 (8)            |               | "           | 85    | 0     | 116    |                   |
|            | 9   | C (6)            | 2 (4)         | 660         | 135   | 135   | 98     | Curve 4           |
|            |     | C (6)            |               | 660         | 152   | 146   | 100    |                   |
| 10         | 3   | 3 (4)            | "             | 520         | 80    | 0     | 94     |                   |
|            |     | 3 (8)            |               | 520         | 88    | 0     | 90     |                   |
|            | 10  | C (6)            | 3 (4)         | 660         | 118   | 130   | 94     |                   |
|            |     | C (6)            |               | 660         | 118   | 140   | 94     |                   |
| 11         | G   | G (1)            | "             | 634         | 60    | 30    | 94     | Fig.5<br>Curve 13 |
|            |     | G (2)            |               | 640         | 76    | 43    | 90     |                   |
|            |     | G (4)            |               | 640-<br>645 | 78    | 66    | 85     |                   |
|            | 11  | G (2)            | "             | 655         | 82    | 60    | 90     |                   |
|            |     | G (2)            |               | 655         | 82    | 73    | 90     |                   |

Table II - Continued

| Exper-<br>imen-<br>tal<br>No. | Ex-<br>am-<br>ple<br>No. | Sensitizing dye-<br>Amount of dye<br>added<br>( $10^{-5}$ mol/kg of<br>emulsion) | Emul-<br>sion | Maximum<br>sensi-<br>tization<br>(nm) | Rel-<br>ative<br>white<br>light<br>sensi-<br>tivity | Rel-<br>ative<br>red<br>sensi-<br>tivity | In-<br>trin-<br>sic<br>sensi-<br>tivity | Spec-<br>tro-<br>gram |
|-------------------------------|--------------------------|----------------------------------------------------------------------------------|---------------|---------------------------------------|-----------------------------------------------------|------------------------------------------|-----------------------------------------|-----------------------|
| 12                            |                          | D (6)                                                                            | AgBr<br>/I    | 660                                   | 105                                                 | 150                                      | 85                                      |                       |
|                               |                          | D (8)                                                                            |               | " 660                                 | 112                                                 | 160                                      | 80                                      |                       |
|                               |                          | 5 (2)                                                                            |               | " 500                                 | 80                                                  | 0                                        | 100                                     |                       |
|                               |                          | 5 (4)                                                                            |               | " 500                                 | 90                                                  | 0                                        | 100                                     |                       |
|                               |                          | 5 (8)                                                                            |               | " 500                                 | 94                                                  | 0                                        | 104                                     |                       |
|                               | 12                       | D (6)                                                                            | 5 (4)         | " 660                                 | 140                                                 | 170                                      | 85                                      |                       |
|                               |                          | D (6)                                                                            |               | " 658                                 | 145                                                 | 175                                      | 100                                     |                       |
| 13                            |                          | F (2)                                                                            | "             | 650                                   | 73                                                  | 45                                       | 98                                      |                       |
|                               |                          | F (4)                                                                            |               | " 650                                 | 95                                                  | 60                                       | 98                                      |                       |
|                               |                          | F (8)                                                                            |               | " 650                                 | 98                                                  | 60                                       | 95                                      |                       |
|                               | 13                       | F (4)                                                                            | 5 (4)         | " 640                                 | 108                                                 | 100                                      | 100                                     |                       |
|                               |                          | F (4)                                                                            |               | " 640                                 | 108                                                 | 76                                       | 100                                     |                       |
| 14                            |                          | 4 (4)                                                                            | "             | 500                                   | 80                                                  | 0                                        | 100                                     | Fig.5                 |
|                               |                          | 4 (8)                                                                            |               | " 500                                 | 83                                                  | 0                                        | 104                                     | Curve 12              |
|                               | 14                       | F (4)                                                                            | 4 (4)         | " 642                                 | 110                                                 | 88                                       | 94                                      |                       |
|                               |                          | F (4)                                                                            |               | " 642                                 | 110                                                 | 83                                       | 104                                     |                       |
|                               | 15                       | G (2)                                                                            | 4 (4)         | 640-<br>660                           | 80                                                  | 54                                       | 90                                      | Curve 14              |
|                               |                          | G (2)                                                                            |               |                                       | 85                                                  | 70                                       | 90                                      |                       |
| 16                            |                          | K (2)                                                                            | "             | 600                                   | 75                                                  | 30                                       | 94                                      |                       |
|                               |                          | K (4)                                                                            |               | " 630                                 | 90                                                  | 85                                       | 94                                      |                       |
|                               |                          | K (8)                                                                            |               | " 630                                 | 110                                                 | 105                                      | 90                                      |                       |
|                               | 16                       | K (4)                                                                            | 6 (4)         | " 630                                 | 135                                                 | 100                                      | 100                                     | Fig.3                 |
|                               |                          | K (8)                                                                            |               | " 630                                 | 148                                                 | 110                                      | 100                                     | Curve 7               |
|                               | 17                       | H (1)                                                                            | "             | 686                                   | 80                                                  | 164                                      | 88                                      |                       |
|                               |                          | H (2)                                                                            |               | " 686                                 | 85                                                  | 172                                      | 82                                      |                       |
|                               |                          | H (4)                                                                            |               | " 686                                 | 85                                                  | 188                                      | 60                                      |                       |
|                               |                          | H (1)                                                                            | 2 (4)         | 684                                   | 90                                                  | 210                                      | 90                                      |                       |
|                               | 17                       | H (1)                                                                            | 2 (8)         | 684                                   | 94                                                  | 210                                      | 104                                     | Curve 8               |
|                               |                          | H (1)                                                                            | 5 (4)         | 686                                   | 90                                                  | 208                                      | 94                                      |                       |
| 18                            | 18                       | H (1)                                                                            | 5 (8)         | " 686                                 | 90                                                  | 170                                      | 98                                      |                       |

Table II-Continued

| Exper-<br>imen-<br>tal<br>No. | Ex-<br>am-<br>ple<br>No. | Sensitizing dye-<br>Amount of dye<br>added<br>( $10^{-5}$ mol/kg of<br>emulsion) | Emul-<br>sion | Maximum<br>sensi-<br>tization<br>(nm) | Rel-<br>ative<br>white<br>light<br>sensi-<br>tivity | Rel-<br>ative<br>red<br>sensi-<br>tivity | In-<br>trin-<br>sic<br>sensi-<br>tivity | Spec-<br>tro-<br>gram |
|-------------------------------|--------------------------|----------------------------------------------------------------------------------|---------------|---------------------------------------|-----------------------------------------------------|------------------------------------------|-----------------------------------------|-----------------------|
| 19                            |                          | I (4)                                                                            | AgBr<br>/I    | 650                                   | 80                                                  | 120                                      | 86                                      |                       |
|                               |                          | I (6)                                                                            |               | "                                     | 650                                                 | 85                                       | 135                                     | 82                    |
|                               |                          | I (8)                                                                            |               | "                                     | 650                                                 | 85                                       | 140                                     | 75                    |
| 19                            | I (6)                    | I (4)                                                                            | "             | 650                                   | 96                                                  | 152                                      | 90                                      |                       |
|                               | I (6)                    | I (8)                                                                            |               | 650                                   | 110                                                 | 178                                      | 104                                     |                       |
| 20                            |                          | E (2)                                                                            | "             | 650                                   | 90                                                  | 73                                       | 92                                      |                       |
|                               |                          | E (4)                                                                            |               | 650                                   | 96                                                  | 88                                       | 88                                      |                       |
|                               |                          | E (8)                                                                            |               | 650                                   | 100                                                 | 104                                      | 85                                      |                       |
| 20                            | E (4)                    | 5 (4)                                                                            | "             | 650                                   | 108                                                 | 94                                       | 94                                      |                       |
|                               | E (8)                    | 5 (4)                                                                            |               | 650                                   | 110                                                 | 110                                      | 98                                      |                       |
| 21                            |                          | 10(4)                                                                            | "             | 540                                   | 85                                                  | 0                                        | 106                                     |                       |
|                               |                          | 10(8)                                                                            |               | 540                                   | 96                                                  | 0                                        | 110                                     |                       |
| 21                            | L (4)                    | 10(4)                                                                            | "             | 628                                   | 120                                                 | 72                                       | 96                                      |                       |
|                               | L (8)                    | 10(4)                                                                            |               | 628                                   | 138                                                 | 108                                      | 94                                      |                       |
| 22                            | 22                       | L (4)                                                                            | 10(4)         | 628                                   | 146                                                 | 108                                      | 96                                      |                       |
|                               |                          |                                                                                  | 11(4)         |                                       |                                                     |                                          |                                         |                       |
| 23                            |                          | A (6)                                                                            | "             | 632                                   | 120                                                 | 120                                      | 86                                      |                       |
|                               |                          | C(0.3)                                                                           |               |                                       |                                                     |                                          |                                         |                       |
| 23                            | A (6)                    | I (4)                                                                            | "             | 632                                   | 152                                                 | 152                                      | 108                                     |                       |
|                               |                          | C(0.3)                                                                           |               |                                       |                                                     |                                          |                                         |                       |
| 24                            | 24                       | A (6)                                                                            | I (4)         | 630                                   | 178                                                 | 152                                      | 102                                     |                       |
|                               |                          | C(0.3)                                                                           | 11(2)         |                                       |                                                     |                                          |                                         |                       |
| 25                            |                          | H (1)                                                                            | "             | 670                                   | 108                                                 | 260                                      | 86                                      |                       |
|                               |                          | I (4)                                                                            |               |                                       |                                                     |                                          |                                         |                       |
| 25                            | H (1)                    | 7 (4)                                                                            | "             | 670                                   | 124                                                 | 268                                      | 100                                     |                       |
|                               |                          | I (4)                                                                            |               |                                       |                                                     |                                          |                                         |                       |
| 26                            | H (1)                    |                                                                                  | "             | 680                                   | 100                                                 | 164                                      | 84                                      |                       |
|                               | A (4)                    |                                                                                  |               |                                       |                                                     |                                          |                                         |                       |
| 26                            | H (1)                    | 6 (4)                                                                            | "             | 680                                   | 120                                                 | 178                                      | 98                                      |                       |
|                               | A (4)                    |                                                                                  |               |                                       |                                                     |                                          |                                         |                       |
| 27                            | H (1)                    |                                                                                  | "             | 680                                   | 118                                                 | 200                                      | 82                                      |                       |
|                               | B (4)                    |                                                                                  |               |                                       |                                                     |                                          |                                         |                       |
| 27                            | H (1)                    | I (4)                                                                            | "             | 680                                   | 140                                                 | 234                                      | 96                                      |                       |
|                               | B (4)                    |                                                                                  |               |                                       |                                                     |                                          |                                         |                       |

In the aforementioned table, the white light sensitivity and the red sensitivity are given relative to the corresponding sensitivities obtained by exposing to the said daylight source without a filter or through a red filter using a sample containing  $4 \times 10^{-5}$  mol/kg of emulsion of the sensitizing dye C, being calculated as 100. The intrinsic sensitivity is given relative to the sensitivity obtained by exposing the starting emulsion through a blue filter, being calculated as 100.

As is obvious from the result given in Table 2, the white light sensitivity and the red light sensitivity obtained by the combined use of the sensitizing dyes of this invention are far higher than those obtained by the independent use thereof.

As is shown in Examples Nos. 2, 3 and 22 in Table 2, the sensitizing effect obtained by the combination of at least one of the carbocyanine dyes and at least one of the merocyanine dyes is not deteriorated if an orthochromatic sensitizing dye already known, such as that of 11 or 12, is further used together. The orthochromatic sensitizing dyes used together with the sensitizing dyes employed in this invention are, for example, 2,2'-cyanine and pseudo-type cyanine (e.g., 2'-thiacyanine) having the following chemical structures, but are not solely limited to these.



Although the present invention has been adequately discussed above in the foregoing specification and examples, it is readily apparent that various changes and modifications can be made without departing from the spirit and scope thereof.

What is claimed is:

1. A silver halide photographic emulsion comprising a supersensitizing combination of at least one sensitizing carbocyanine dye having two heterocyclic nuclei selected from the group consisting of a benzothiazole nucleus, a benzoselenazole nucleus, a  $\beta$ -naphthoselenazole nucleus and a  $\beta$ -naphthothiazole nucleus, the meso-position of said dye being substituted with a member selected from the group consisting of a methyl and an ethyl group, and at least one merocyanine dye in which a tetrazole derivative nucleus and a merocyanine nucleus are connected through a dimethine chain.

2. The silver halide photographic emulsion of claim 1, wherein at least one of the N-substituents of the heterocyclic nuclei of the carbocyanine dye is a member selected from the group consisting of a sulfoalkyl and a carboxyalkyl group.

3. The silver halide photographic emulsion of claim 1, wherein the carbocyanine dye is represented by the following formula (I) and the merocyanine dye by the following general formula (II):



wherein  $R_1$  and  $R_2$  each represents a lower alkyl group;  $A$  represents a member selected from the group consisting of a methyl and an ethyl group;  $Z_1$  and  $Z_2$  represent nonmetallic atoms necessary to complete a ring selected from the group consisting of a benzothiazole nucleus, a benzoselenazole nucleus, a  $\beta$ -naphthoselenazole nucleus, and a  $\beta$ -naphthothiazole nucleus;  $X_1$  represents an anion; and  $m$  represents 0 or 1, provided that  $m = 0$  when an intermolecular salt is formed:



wherein  $R_3$  and  $R_4$  each represents a lower alkyl group;  $B$  represents a member selected from the group consisting of a lower alkyl and an aryl group;  $Z_3$  represents a member selected from the group consisting of  $=N-R_5$ , an oxygen atom, and a sulfur atom;  $R_5$  being a lower alkyl group.

4. The silver halide photographic emulsion of claim 3, wherein  $Z_3$  of the formula (II) is an oxygen atom.

5. The silver halide photographic emulsion of claim 4, wherein  $Z_1$  and  $Z_2$  of formula (I) are nonmetallic atoms necessary to complete a member selected from the group consisting of a benzothiazole and a  $\beta$ -naphthothiazole nucleus.

6. The silver halide photographic emulsion of claim 3, wherein  $A$  of formula (I) is a methyl group and  $Z_3$  of formula (II) is a sulfur atom.

7. The silver halide photographic emulsion of claim 1, wherein the emulsion further contains at least one orthochromatic sensitizing dye.

8. The silver halide photographic emulsion of claim 7, wherein the orthochromatic sensitizing dye is selected from the group consisting of a 2,2'-cyanine dye and a pseudo-type cyanine dye.

9. The silver halide photographic emulsion of claim 45 1, wherein the carbocyanine dye is selected from the group consisting of



19



and



20



and the merocyanine dye is selected from the group consisting of

10. The silver halide photographic emulsion of claim 7, wherein the orthochromatic sensitizing dye is selected from the group consisting of



and



11. A silver halide photographic emulsion comprising a supersensitizing combination of



and



12. The silver halide photographic emulsion comprising a supersensitizing combination of



and

5



10 13. The silver halide photographic emulsion comprising a supersensitizing combination of

15



20 and

25



30 14. The silver halide photographic emulsion comprising a supersensitizing combination of

35



and

40



45

15. The silver halide photographic material comprising a layer containing the silver halide emulsion of claim 1.

50 16. The silver halide photographic emulsion of claim 1, wherein the mol ratio of said carbocyanine dye to said merocyanine dye ranges from 9:1 to 1:9.

55 17. The silver halide photographic emulsion of claim 1, wherein each of said cyanine and merocyanine dye is present in an amount of  $1 \times 10^{-6}$  to  $1 \times 10^{-3}$  mol per mol of silver.

\* \* \* \* \*